

April 2, 1940.

T. B. CHACE

2,195,614

METHOD OF AND MEANS FOR PRODUCING COMPOSITE METAL PRODUCTS

Filed Feb. 7, 1938

Fig. 1.



Fig. 2.



Fig. 5.



Fig. 3.



Fig. 4.



Inventor:  
Thomas B. Chace.

By *Proteracum Bottlers, Inc.*

Attty:

## UNITED STATES PATENT OFFICE

2,195,614

METHOD OF AND MEANS FOR PRODUCING  
COMPOSITE METAL PRODUCTS

Thomas B. Chace, Winnetka, Ill.

Application February 7, 1938, Serial No. 189,097

18 Claims. (Cl. 22—203)

My invention relates generally to mould constructions, and it has particular relation to the moulds used in the production of composite metal slabs which may be rolled into various shapes and sizes. This application is a continuation-in-part of my copending application, Serial No. 142,387, filed May 13, 1937, which is a continuation in part of my copending applications, Serial No. 6,497, filed February 14, 1935, now Patent 2,145,-  
10 248, and Serial No. 64,280, filed February 17, 1936.

In the bonding to steel of some high corrosion resistant alloys and the subsequent rolling of the composite slab, the design and type of mould is very important in making the process commercial and the product usable. Some of the copper alloys, such as silicon copper, are particularly fluid in the molten state and are very difficult to hold, in the molten state, on the surface of the steel backing slab. Some of the other non-corrosive alloys, such as the high nickel coppers of from 20% to 40% nickel content, having melting temperatures up to 2400° F., or Monel metal or stainless steel, having melting temperatures similar to the steel backing slab, are difficult to hold in the molten state because of the extremely high casting temperatures involved. The mould must be liquid-tight after having been preheated to temperatures of around 2200° F.

Large slabs having a thickness of 10" to 12" must be preheated for five or six hours at this temperature, and the mould forming a part thereof must be such that it will not burn out and will remain liquid-tight as a container for the molten flux during the preheating, as well as a container for the non-corrosive metal which is cast in the mould after preheating. This casting operation differs from ordinary casting in that the mould, in some cases, is preheated to a temperature above the melting point of the casting alloy and, since the base of the mould or backing member is made up of a relatively thick steel slab, the heat is maintained for a considerable period and the cast metal remains molten much longer than ordinary cast metal, remains molten in a cold mould, in which case the cast metal solidifies quickly. In fact, for the cladding of some combinations, such for example as my silicon-copper alloys, it is necessary to prolong the molten state of the casting alloy to perfect a bond between the two.

In view of the foregoing, an object of my invention is the provision of a mould which can be rolled as a part of a composite slab, either directly from the bonding heat or as soon as the cast

metal has solidified and cooled to the maximum hot rolling temperature.

Another object of my invention is to provide an open-faced mould on which the depth and width can be readily regulated as the measuring means for determining the required thickness of the cast alloy in proportion to the steel backing metal.

Another object of my invention is to provide an open-faced mould that can be used to clad a relatively large surface of a slab of base metal and to leave only a small surface of the cladding metal exposed while the mould is being filled and when the cladding metal is freezing.

Another object of my invention is to provide an open-faced mould formed by a slab of base metal and a thin metal mould member, which mould will be liquid tight and such that the mould filling metal will not bond to the thin metal mould member.

Another object of my invention is to provide an open-faced mould by means of which a slab of base metal can be cladded on opposite surfaces with different cladding metals, such as a copper alloy on one surface and nickel or stainless steel on the other surface.

A further object of my invention is to provide an open-faced mould construction that can be readily adapted to fit any size of slab or backing material.

Another object of my invention is to provide an open-faced mould which may be elongated in working, such as rolling, and which will maintain a uniform rolled edge.

Other objects of my invention will, in part, be obvious and in part appear hereinafter.

Accordingly, my invention is disclosed in the embodiments hereof shown in the accompanying drawing, and it comprises the features of construction, combination of elements and arrangement of parts which will be exemplified in the description hereinafter set forth and the scope of the application of which will be indicated in the appended claims.

For a more complete understanding of the nature and scope of my invention reference may be had to the following detailed description, taken in connection with the accompanying drawing, in which:

Figure 1 is a sectional view showing one form of mould construction for producing a slab with a layer of cladding metal on opposite sides;

Figure 2 is a sectional view taken along the line 2—2 of Figure 1;

Figure 3 is a fragmentary perspective view of another mould construction for producing a com-

posite slab having a layer of cladding metal on the top and end surfaces;

Figure 4 is a sectional view taken along the line 4—4 of Figure 3; and

5 Figure 5 is a sectional view showing one form of mould construction for producing a slab with a layer of cladding metal on a large lateral surface and the bottom of the mould being closed by resting the mould construction on a foundry floor.

10 The utility and construction of my type of mould for the purpose of cladding by casting one metal or different metals on opposite surfaces of another, or on the upper surface in combination with other surfaces, are of great importance.

15 For instance, any size of slab or backing member may be chosen with respect to starting and finished size which best fits the requirements of a particular order or specification with a minimum scrap loss. This permits using regular bloom

20 sections requiring a minimum of processing before cladding. If the clad slab is to be rolled into plates, for instance, and if the facing or casting alloy has similar compression resistance to the steel backing material so that they roll evenly,

25 the steel strips and channel-shaped members are welded to the sides and ends, leaving the full area of the slab for cladding, thus producing a minimum of scrap loss. If the bloom has irregular edges and ends, so that welding along the edges 30 and ends is not practical, the mould members can be located on the upper and side surfaces of the bloom, leaving the irregular ends and edges extending on the outside of the mould members.

35 It will be understood that the different conditions will govern the particular type of mould construction that is employed.

There are some cases in which it is desirable to clad a base metal slab on opposite surfaces with different metals. In the application of

40 cladded metal to heat exchangers, condenser tubes and other industrial uses, the cladded metal may be exposed to a different condition on one surface than it is on the other. Hence it is desirable to clad the opposite surfaces with

45 metals or alloys suitable to the conditions under which they are to be used. In some cases it might be desirable to have a copper alloy on one surface and stainless steel or a nickel alloy on the other. Mould constructions and methods are de- 50 scribed hereinafter which can be used to clad a slab of base metal on opposite surfaces with the same or different metals.

Referring to Figures 1 and 2, there is shown a mould construction by which opposite surfaces of a slab may be clad. As therein illustrated, a mould construction is provided for cladding the opposite surfaces 27 and 28 of a slab of base metal 29. For this purpose relatively thin metal mould members 30 are provided, having inturned end 55 and side portions 31 and 32 that may be welded to the adjacent sides and end of the slab 29, as indicated at 33 and 34, respectively. The mould spaces thus formed may be filled with a suitable flux and then the mould may be pre-heated to bring it up to the desired temperature. The mould spaces may then be filled with the desired cladding metal to provide, on cooling, a composite slab with integrally bonded layers of cladding metal on the opposite surfaces 27 and 70 28. The inturned bottoms 31 may be omitted and the mould construction be set on the sand floor of the foundry so as to close the bottom of the mould spaces.

The mould construction shown in Figures 1 75 and 2 may be lined with a non-binding material

and used in the same manner as is the mould construction shown in Figure 5 and described hereinafter. This will allow the removal of the mould members 30 and expose the surfaces of the cladding metal.

The mould spaces in Figures 1 and 2 may be filled with different metals rather than with the same metal. This will provide slab 29 with different cladding metals on its surfaces 27 and 28. For example, the surface 27 may be clad with a 1 cuprous metal and surface 28 may be clad with nickel or stainless steel.

If the bottoms of the mould spaces are not closed by inturned projections 31 as shown in Figure 1 but are closed by a sand floor, this will 1 allow the base metal slab to be heated in a molten bath of slag. When the slab is withdrawn, the slag will run out of the mould space and a thin coating of slag will adhere to the surface of the slab and to the surface of the mould members 30, thereby preventing oxidation. When the mould is poured, this coating will fuse and be displaced by cladding metal.

In Figures 3 and 4 of the drawing a mould construction is illustrated that may be employed 2 for cladding the top surface 37 and end surfaces 38 of a base metal slab 39. For this purpose relatively thin side members 40 are welded, as indicated at 41, to the top surface 37 along its edges. Relatively thin metal mould members 42, 3 having inturned sides 43 and bottoms 44, are spaced from the end surfaces 38, as shown, and are welded to the side and bottom surfaces of the slab 39, as indicated at 45 and 46. The in-turned bottoms 44 may be omitted and the mould 4 construction set on the casting floor so that the bottom is closed thereby. After the mould members 40 and 42 have been welded in place, as illustrated, a mould space is then formed by the side members 40, the mould members 42 and the 4 surfaces 37 and 38, into which the cladding metal 5 may be poured as desired. Alternatively, slabs of cladding metal may be disposed in the mould spaces thus formed and the entire combination heated up to the welding temperature.

For the purpose of definitely limiting the depth of cladding metal above the top surface 37, the mould members 42 may be provided with cut-away sections 47 through which the molten 6 cladding metal may escape.

In Figure 5 a mould construction is illustrated which may be used to clad a large surface 48 of a base metal slab 50. The bottom 51 of the mould is shown as being closed by a foundry floor 52. Using the floor 52 to close the mould 7 may, in some cases, be desirable rather than closing the mould by inturning a projection on the base of the mould member 53.

The inner surface 54 of mould member 53 is coated or lined with a suitable material 55 such as a fire clay or an aluminum oxide base to form a non-bonding surface to be contacted by the cladding metal. This non-bonding surface may be provided by oxidizing the inner surface 54 of the mould member 53 so that a scale will be formed thereupon. The inner surface 54 may be lined or coated with some refractory material such as the fire clay used to line furnaces and crucibles in foundries. Magnesia, as an insulator or non-bonding layer, may be deposited upon the inner surfaces when bonding is to be prevented. This may be deposited by means of a wash, like whitewash. Sodium silicate may be employed to attach a layer of powdered material to the selected surfaces. By so coating or lining the inner

surface 54 it will be possible to remove the mould member 53 after the cladding metal has frozen, as by cutting it away with a torch, and thus have a clean surface of cladding metal exposed. If a suitable bond-preventing layer is provided, the slab may be rolled through a desired stage or stages without removal of the mould 53.

The mould member 53 is substantially channel-shaped. It is welded on the base metal slab 50 on opposite sides in the same manner that mould members 30 in Figures 1 and 2 are welded to the base metal slab 28 at 23. The sand upon which it is set effectively seals the lower end of the mould.

15 The mould construction illustrated in Figure 5 has valuable advantages in cladding a base metal slab with certain cladding metals. It is readily seen from Figure 5 that only a small surface of the cladding metal will be exposed when the metal is poured and after it solidifies. The small surface that is exposed will be on an end of the slab 50 and may be cropped or cut off with little loss.

25 Some of the alloys and metals used for cladding are subject to rapid oxidation and gas absorption at the temperatures used for cladding. Certain metals, like copper, tend to squeeze out absorbed gases on freezing, and form rough surfaces as a result. A small amount of silicon, as 30 low as 0.1% or even less, tends to limit this gas absorption. Using the mould construction as shown in Figure 5 the cladding metal may be subjected to high temperatures over long periods, and oxidation and gas absorption will be limited 35 to the small surface on the top of the mould. After the mould has cooled as much as desired the mould member 53 may be removed and a clean and smooth surface of cladding metal will be obtained.

40 Since certain further changes may be made in the foregoing mould constructions, and different embodiments of the invention may be made without departing from the scope thereof, it is intended that all matter shown in the accompanying drawing or described hereinbefore shall be interpreted as illustrative and not in a limiting sense.

I claim as my invention:

1. Means for producing a composite slab comprising, a slab of base metal of uniform thickness, and a pair of relatively thin metal members welded to said slab on opposite sides in such manner as to form moulds of substantially uniform width with adjacent surfaces of said slab for retaining cladding metal therein in the molten state whereby, on cooling, said slab is provided with integrally bonded layers of cladding metal of substantially uniform thickness on said surfaces.

- 60 2. Means for producing a composite slab comprising, a slab of base metal of uniform thickness, and a pair of relatively thin metal channel-shaped members welded to said slab on opposite sides in such manner as to form moulds of substantially uniform width with adjacent surfaces of said slab for retaining cladding metal therein in the molten state whereby, on cooling, said slab is provided with integrally bonded layers of cladding metal of substantially uniform thickness on said surfaces.
- 65
- 70

3. Means for producing a composite slab comprising, a slab of base metal of uniform thickness, and a pair of relatively thin metal channel-shaped members welded to said slab on opposite vertical sides in such manner as to form moulds

of substantially uniform width with adjacent vertical surfaces of said slab for retaining cladding metal therein in the molten state whereby, on cooling, said slab is provided with integrally bonded layers of cladding metal of substantially uniform thickness on said surfaces, the lower ends of said channel-shaped members being turned inwardly toward and welded to the bottom surface of said slab. 3

4. Means for producing a composite slab comprising, a slab of base metal of uniform thickness, and a relatively thin metal member welded to opposite sides of said slab so as to form a mould of substantially uniform width with the adjacent surface of said slab for retaining cladding metal therein in the molten state whereby, on cooling, said slab is provided with an integrally bonded layer of cladding metal of substantially uniform thickness on said surface. 10 15

5. Means for producing a composite slab comprising, a slab of base metal of uniform thickness, and a relatively thin metal channel-shaped member welded to opposite sides of said slab so as to form a mould of substantially uniform width with the adjacent surface of said slab for retaining cladding metal therein in the molten state whereby, on cooling, said slab is provided with an integrally bonded layer of cladding metal of substantially uniform thickness on said surface. 20 25 30

6. Means for producing a composite slab comprising, a slab of base metal of uniform thickness, and a relatively thin metal channel-shaped member welded to said slab on opposite vertical sides in such manner as to form a mould of substantially uniform width with the adjacent vertical surface of said slab for retaining cladding metal therein in the molten state whereby, on cooling, said slab is provided with an integrally bonded layer of cladding metal of substantially uniform thickness on said surface, the lower end of said channel-shaped member being turned inwardly toward and welded to the bottom surface of said slab. 35 40

45  
7. Means for producing a composite slab comprising, a slab of base metal, a pair of relatively thin metal end members welded to opposite sides of said slab and spaced from the end surfaces thereof, and a pair of relatively thin metal side members welded along opposite sides of said slab and projecting above the top surface thereof, said end and side members with the end and top surfaces of said slab forming a mould for retaining cladding metal therein in the molten state whereby, on cooling, said slab is provided with an integrally bonded layer of cladding metal on said end and top surfaces.  
50  
55

8. Means for producing a composite slab comprising, a slab of base metal, a pair of relatively thin metal channel-shaped end members welded to opposite sides of said slab and spaced from the end surfaces thereof, and a pair of relatively thin metal side members welded along opposite sides of said slab and projecting above the top surface thereof, said end and side members with the end and top surfaces of said slab forming a mould for retaining cladding metal therein in the molten state whereby, on cooling, said slab is provided with an integrally bonded layer of cladding metal on said end and top surfaces. 70

9. Means for producing a composite slab comprising, a slab of base metal, a pair of relatively thin metal channel-shaped end members welded to opposite vertical sides of said slab and spaced from the vertical end surfaces thereof, and a

pair of relatively thin metal side members welded along opposite vertical sides of said slab and projecting above the top surface thereof, said end and side members with the end and top surfaces of said slab forming a mould for retaining cladding metal therein in the molten state whereby, on cooling, said slab is provided with an integrally bonded layer of cladding metal on said end and top surfaces, the lower ends of said channel-shaped end members being turned inwardly toward and welded to the bottom surface of said slab.

10. Means for producing a composite slab comprising, a slab of base metal, a pair of relatively thin metal channel-shaped end members welded to opposite sides of said slab and spaced from the end surfaces and projecting above the top surface thereof, and a pair of relatively thin metal side members interfitting with the angles formed by the flanges and beds of said channel-shaped members and welded along opposite edges of the top surface of said slab and to said channel-shaped members, said end and side members with end and top surfaces of said slab forming a mould for retaining cladding metal therein in the molten state whereby, on cooling, said slab is provided with integrally bonded layers of cladding metal on said end and top surfaces.

11. Means for producing a composite slab comprising, a slab of base metal, a pair of relatively thin metal channel-shaped end members welded to opposite sides of said slab and spaced from the end surfaces and projecting above the top surface thereof, and a pair of relatively thin metal side members interfitting with the angles formed by the flanges and beds of said channel-shaped members and welded along opposite edges of the top surface of said slab and to said channel-shaped members, said end and side members with end and top surfaces of said slab forming a mould for retaining cladding metal therein in the molten state whereby, on cooling, said slab is provided with integrally bonded layers of cladding metal on said end and top surfaces, the lower ends of said channel-shaped end members being turned inwardly toward and welded to the bottom surface of said slab.

12. Means for producing a composite slab comprising, a slab or block of base metal of uniform thickness, and a substantially channel-shaped housing or closure welded to a vertical surface of said slab so as to provide a vertical mould space of substantially uniform width into which cladding metal may be introduced to produce a bonding of the cladding metal to said vertical surface of said slab and which after completion of said cladding operation can be rolled as part of the composite slab formed.

13. Means for producing a composite slab comprising, a slab of base metal, and a relatively thin metal member welded to opposite vertical sides of said slab so as to form a mould space

with the adjacent surface of said slab for retaining cladding metal therein in the molten state whereby, on cooling, said slab is provided with an integrally bonded layer of cladding metal on said surface, the inner surface of said thin metal member being lined with a non-bonding material.

14. Means for producing a composite slab comprising, a slab of base metal, and a relatively thin metal channel-shaped member welded to opposite vertical sides of said slab so as to form a mould space with the adjacent surface of said slab for retaining cladding metal therein in the molten state whereby, on cooling, said slab is provided with an integrally bonded layer of cladding metal on said surface, the inner surface of said thin metal channel-shaped member being lined with a non-bonding refractory material.

15. The method of producing a composite slab which comprises, welding a relatively thin channel-shaped metal member to opposite vertical sides of a relatively thick slab of base metal to form a vertical mould space with the adjacent vertical surface of said slab, lining the inner surface of the channel-shaped mould member with a non-bonding material, and filling said mould space with cladding metal.

16. The method of producing a composite slab which comprises, welding a relatively thin channel-shaped metal member to opposite vertical sides of a relatively thick slab of base metal to form a vertical mould space with the adjacent vertical surface of said slab, lining the inner surface of the channel-shaped mould member with a non-bonding material, filling said mould space with cladding metal, allowing the cladding metal to solidify, and removing the mould member to expose the surface of the cladding metal.

17. The method of producing a composite slab which comprises, welding thin metal channel-shaped members to opposite vertical sides of a relatively thick slab of base metal to form vertical mould spaces with the adjacent vertical surfaces of said slab, lining the inner surfaces of the channel-shaped mould members with a non-bonding material, and filling each vertical mould space with a different cladding metal.

18. The method of producing a composite slab which comprises, welding thin metal channel-shaped members to opposite vertical sides of a relatively thick slab of base metal to form vertical mould spaces with the adjacent vertical surfaces of said slab, lining the inner surfaces of the channel-shaped mould members with a non-bonding material, filling one vertical mould space with cuprous cladding metal and the other vertical mould space with stainless steel, allowing the cladding metals to solidify, and removing the mould members to expose the vertical surfaces of cuprous or stainless steel cladding metals.

THOMAS B. CHACE.